

## 1

3,497,531

STABILIZATION OF OXIRANE CONTAINING  
FATTY DERIVATIVES

Rex J. Sims, Pleasantville, N.Y., assignor to Swift & Company, Chicago, Ill., a corporation of Illinois  
No Drawing. Continuation of application Ser. No. 166,420, Jan. 15, 1962. This application Nov. 25, 1966, Ser. No. 597,171  
Int. Cl. C07d 1/00; C08f 45/58

U.S. Cl. 260—348

3 Claims

10

## ABSTRACT OF THE DISCLOSURE

Fatty, oxirane-containing compounds stabilized against loss of oxirane oxygen by the presence of phenolic fat antioxidants such as propyl gallate.

This application is a continuation of application Ser. No. 166,420, filed Jan. 15, 1962 and now abandoned.

This invention relates to the stabilization of oxygen-containing fatty derivatives and, more particularly, to stabilized oxirane-containing higher fatty derivatives protected against loss of oxirane oxygen and increases in acidity.

Oxirane-substituted higher fatty acids, higher fatty alcohols, higher fatty acid amides, and higher fatty acid esters are valuable compositions, particularly the esters of oxirane-substituted higher fatty acids and esters of oxirane-substituted higher fatty alcohols and the value of these compositions is attributable in many cases to the oxirane oxygen content of the composition. Oxirane-containing higher fatty acid esters, for example, have been found of significant value as plasticizer-stabilizers for halogen-containing compositions such as the vinyl halide resins.

Oxirane-containing glyceride oils and epoxidized fatty acid esters of mono-, di-, and polyhydric alcohols generally are employed widely as plasticizer-stabilizers in synthetic resins. These epoxy esters inhibit degradation of the vinyl resin and this inhibition has been attributed to the presence of the oxirane group. Also, the presence of the oxirane group in the ester appears to promote compatibility of the ester with resins.

These oxirane-substituted higher fatty derivatives undergo certain changes upon long periods of storage and when the materials are subjected to elevated temperature and/or pressure as is encountered in the processing of resins with which they are formulated. These changes include an increase in acidity of the oxirane-containing material and a development of an objectionable odor and loss of epoxy oxygen accompanied by lessening of stabilizing properties and poorer compatibility with resins.

It is accordingly an object of this invention to stabilize oxirane-containing higher fatty derivatives against loss of oxirane oxygen and odor development and also preserve the stabilizing properties and compatibility of such derivatives with resins.

A further object of the invention is the provision of oxirane-containing higher fatty derivatives stabilized against decreases in oxirane oxygen content.

Another object of the invention is the provision of synthetic plastics containing stabilized oxirane-substituted fatty materials which oxirane-substituted fatty materials retain plasticizer and stabilizing efficiency as well as compatibility substantially undiminished after long periods of storage.

Still another object of the invention is the provision of a method for protecting oxirane-substituted higher fatty materials against loss of oxirane oxygen.

## 2

Additional objects, if not specifically set forth herein, will be readily apparent to those skilled in the art from the detailed description of the invention which follows.

Generally, the invention comprises oxirane-containing higher fatty derivatives having embodied therein protective agents for the



group and synthetic plastic compositions containing oxirane-substituted higher fatty materials which plastics can be stored for long periods and/or processed and formulated at elevated temperatures without substantial decrease in oxirane content of the fatty material. Also within the contemplation of the invention are methods for inhibiting and preventing the oxidative degradation of the oxirane-substituted fatty materials and the development of objectionable odors in such materials. The method of the invention involves the embodiment in such oxirane-substituted fatty materials of a protective amount of an organic phenolic composition.

More specifically, the invention provides epoxidized higher fatty acids, aromatic and lower aliphatic alcohol esters of such fatty acids, amides and hydrazides of such fatty acids, as well as esters of oxirane-containing higher fatty alcohols, stabilized against degradation and loss of oxirane oxygen by a small amount of a phenolic fat antioxidant.

While directed to oxirane-containing fatty materials generally, the stabilization is directed particularly to epoxy esters which are employed extensively in plasticizing vinyl halide resins. The oxirane-containing fatty acid derivatives to which the invention is particularly directed are the mono-, di-, tri-, tetra-, and pentahydric alcohol esters of oxirane-containing fatty acids of 7-30 and preferably 10-30 carbons. Esters of such acids with monohydric aliphatic alcohols having 1-18 carbons and esters with dihydric aliphatic alcohols of 2-6 carbons, as well as with aliphatic polyhydric alcohols generally, are contemplated. Suitable monohydric alkyll and alkenyl alcohols providing the alcohol moiety of such esters include methyl, ethyl, propyl, isopropyl, butyl, isobutyl, amyl, isoamyl, hexyl, heptyl, and octyl alcohols. Dihydric alcohols include the lower glycols as ethylene glycol, 1,2-propanediol, 1,3-propanediol, dimethylene glycol, trimethylene glycol, tetramethylene glycol up to and including hexamethylene glycol.

Benzoid alcohols which may be employed in preparing the oxirane-containing fatty acid esters which can be advantageously treated in accordance with the invention are those benzoid alcohols having less than 10 carbons and including benzyl, phenyl, 2-phenylethyl, 1-phenylethyl, and nuclear methylated phenyl alcohols.

The polyhydric alcohol esters of oxirane-containing fatty acids include the tri-, tetra-, penta-, and hexahydric alcohol esters of the fatty acid moiety. Included within this group are those aliphatic alcohols having 3-6 carbons and three or more alcohol groups. These include glycerol, erythritol, pentaerythritol, and hexitols such as mannitol and sorbitol. Mixed oxirane-containing esters such as those disclosed and claimed in U.S. Patent No. 2,978,463, issued Apr. 4, 1961, to F. E. Kuester et al. may also be used.

Highly epoxidized low by-product esters such as those disclosed in co-pending application Ser. No. 807,985, filed Apr. 22, 1959, now U.S. Patent No. 3,117,754, are particularly well suited to treatment in accordance with the invention. These materials because of their high oxirane

content and low hydroxyl and low polymer content are more compatible with vinyl resins than epoxy esters having a lower oxirane content and greater amount of by-products. Because of the low by-product and low polymer content of these materials a higher level of compatibility with the resin is obtained and larger amounts of such esters can be employed in plasticizing a vinyl halide polymer.

The invention has particular application as applied to aliphatic mono- and polyhydric lower alcohol esters of high oxirane higher fatty acids which contain a minimum of by-products such as polymers and hydroxylated esters. Those epoxidized fatty acid esters made from fatty acids having an oxirane content in the range of about 8.8-12.3% oxirane oxygen should have an infrared absorptivity at 2.9 microns (corrected for background) of .020 maximum. Other epoxy esters of fatty acids having an oxirane content of about 5.8-7% oxirane oxygen should have an infrared absorptivity at 2.9 microns (corrected for background) of .01 maximum. High oxirane linseed or perilla oil are examples of glyceride esters characterized by an absorptivity of .02 maximum at 2.9 microns while high oxirane soybean oil and 2-ethylhexyl esters of tall oil fatty acids, among others, have an absorptivity of .01 maximum at 2.9 microns.

The phenolic antioxidants which are known in the art as fat antioxidants provide stabilization of the oxirane-substituted compositions. Antioxidants such as butylated hydroxy anisole, butylated hydroxy toluene, and propyl gallate are representative of the group generally known as fat antioxidants. Commercial butylated hydroxy anisole is a mixture of 3-tertiary butyl-4-hydroxy anisole and 2-tertiary butyl-4-hydroxy anisole. Butylated hydroxy toluene (2,6-ditertiary butyl-p-cresol) is also an article of commerce. It is generally desirable to dissolve the additive or mixture of additives in a mutual solvent such as propylene glycol, ethanol, monoglycerides or like solvent in order to insure distribution of the stabilizer throughout the oxirane-containing composition.

The edible or nontoxic phenolic antioxidants are preferred for use in oxirane-containing esters which are to be used with vinyl halide resins designed for use around foods. The production of food packaging films from polyvinyl chloride requires that the film not contain inedible or toxic ingredients and thus epoxidized oils used in such formulations should contain stabilizers approved for food use. Further when the epoxidized oil is utilized in vinyl halide resins the stabilizer should be a composition which does not adversely affect the vinyl halide. For this reason stabilizers having amino groups are not favored in such formulations. Other suitable antioxidants useful in some applications are beta-naphthol, hydroquinone and compounds such as 2-tertiary butyl-4-decyloxyphenol, 2-tertiary butyl-4-dodecyloxyphenol, 2-tertiary butyl-4-tetradecyloxyphenol and 2-tertiary butyl-4-octadecyloxyphenol. A preferred stabilizer mixture for use in oxirane substituted compositions to be used with polyvinyl chloride resins is as follows:

|                  | Percent by weight |
|------------------|-------------------|
| Propyl gallate   | 20                |
| Citric acid      | 10                |
| Propylene glycol | 70                |

Substitution of gentisic acid for propyl gallate in the above formulation results in an almost equally effective degree of stabilization.

Because the stabilizing efficiency of individual compositions and mixtures of such compositions vary, the amount of stabilizer required depends upon the particular composition employed. Also, the conditions to which the oxirane-containing material is subjected affect the amount of stabilizer required. Usually about .01-0.5% of the stabilizing material based on the weight of the oxirane-containing composition serves to satisfactorily stabilize against increase in acidity of the oxirane-substituted com-

position. Smaller amounts down to around .0025% appear to provide a beneficial result although amounts in the range around .02-.04% appear to be optimum. While larger amounts can be used, up to around 5% without adversely affecting the oxirane compositions, the use of such large amounts may not be desirable inasmuch as the increased protection is not commensurate with the increase in the amount used. In some cases the use of larger amounts is advantageous as where the epoxidized fatty material is employed as a plasticizer-stabilizer for vinyl halide resins. Amounts in the range of 1-3 parts of antioxidant per hundred parts of resin in a vinyl chloride formulation improve processability of the resin and inhibit viscosity build-up.

The method for incorporating the stabilizers in the oxirane-containing derivative or in plastic formulations containing such oxirane derivative is not critical so long as the stabilizer is distributed throughout the mixture and maintained in contact with the oxirane-containing material. The stabilizer can be incorporated in the resin-oxirane-containing composition mixture or the stabilizer can be incorporated in the oxirane-containing material as part of the manufacturing operation producing such material.

Best results in realizing the benefits of the invention are obtained, if the oxirane-containing composition is refined as by caustic refining. If an epoxidized glyceride, for example, is treated with sodium hydroxide, potassium hydroxide or other alkali to remove any acidic materials and/or peroxides, the effect of the stabilizer will be substantially increased. A convenient method for incorporating butylated hydroxy toluene and/or butylated hydroxy anisole in an epoxidized glyceride involves first dissolving the additives in a solvent such as propylene glycol, incorporating the solvent containing the additives in the glyceride oil and subsequently subjecting the oil to a steam deodorization step to remove volatiles which volatiles also include the glycol solvent. Alkali refining prior to addition of the stabilizer insures that no residual inorganic acid possibly employed in the production of the epoxidized composition will be present therein to accelerate degradation on storing.

Accelerated aging tests have been employed to demonstrate the stabilizing effect of the additives of the invention. This accelerated aging test involves placing the sample containing the stabilizer, as well as a control sample with no stabilizer, in 50 gram amounts in open 100 ml. beakers in a laboratory electrically heated oven. The temperature of the oven is adjusted to a given temperature and observations are made after varying lengths of time. Other methods for testing stability of the epoxide can also be used and this method has been selected for simplicity and convenience.

The following examples which are intended to be illustrative and which should not be considered to place any limitation upon the invention, show the stabilizing effect of the phenolic antioxidants.

#### Example I

The oxirane-containing material is epoxidized soybean oil having an oxirane content of 7.02%, an iodine value of 2, a Gardner color of less than 1, and an infrared absorptivity at 2.9 microns (corrected for background) of .01 maximum. This epoxidized soybean oil contains an average of over 4 reactive epoxy groups per molecule. A 50 gram sample of this epoxidized oil containing no stabilizer was compared with 50 gram samples of same oil containing .01% propyl gallate and a sample containing .01% butylated hydroxy anisole and a sample containing .01% butylated hydroxy toluene. The samples were heated in the oven at 85° C. for varying lengths of time up to 28 days and peroxide values, as well as free fatty acid (as acetic acid) and oxirane analyses, were conducted. Table I shows the increase in acidity of the unstabilized sample and the inhibition of this acidity increase by the additives.

TABLE I

| Sample                                             | Percent Free Fatty Acid (as Acetic)<br>After Number of Days Indicated as 85° C. |        |         |         |        |
|----------------------------------------------------|---------------------------------------------------------------------------------|--------|---------|---------|--------|
|                                                    | 0 days                                                                          | 7 days | 14 days | 21 days | 28 day |
| Sample I, epoxidized soybean oil (control)         | .013                                                                            | .027   | .040    | .095    | .166   |
| Sample I containing .01% propyl gallate            | .009                                                                            | .009   | .016    | .030    |        |
| Sample I containing .01% butylated hydroxy anisole | .009                                                                            | .009   | .016    | .035    |        |
| Sample I containing .01% butylated hydroxy toluene | .009                                                                            | .008   | .016    | .052    |        |

Oxirane determinations were made after 14 and 28 days and the results are as follows:

TABLE II

| Sample                                             | Percent Oxirane<br>After Number<br>of days Indicated<br>Indicated at<br>85° C. |      |      |
|----------------------------------------------------|--------------------------------------------------------------------------------|------|------|
|                                                    | 0                                                                              | 14   | 28   |
| Sample I epoxidized soybean oil (control)          | 7.02                                                                           | 6.99 | 6.67 |
| Sample I containing .01% propyl gallate            |                                                                                | 7.10 |      |
| Sample I containing .01% butylated hydroxy anisole | 7.07                                                                           |      |      |
| Sample I containing .01% butylated hydroxy toluene | 7.02                                                                           | 6.97 |      |

## EXAMPLE II

The epoxidized soybean oil employed in the tests recorded in the preceding example was employed to demonstrate the increased effectiveness of butylated hydroxy toluene when added in increasing amounts to such epoxidized oil. 50-gram samples of the oil were placed in 100-milliliter beakers and while one sample containing no added stabilizer was employed as the control, varying amounts of butylated hydroxy toluene were added to the other samples and the increase in acidity and decrease in oxirane content after several days' heating at 85° C. was noted. The results are tabulated in Table III, which

TABLE III

| Sample                                               | Percent Free Fatty Acid (as Acetic)<br>After Number of Days Indicated as 85° C. |        |         |         |         |
|------------------------------------------------------|---------------------------------------------------------------------------------|--------|---------|---------|---------|
|                                                      | 0 days                                                                          | 7 days | 14 days | 21 days | 28 days |
| Sample I, epoxidized soybean oil (control)           | .0125                                                                           | .0338  | .074    | .084    | .129    |
| Sample I containing .0025% butylated hydroxy toluene |                                                                                 | .0303  | .054    | .075    | .103    |
| Sample I containing .005% butylated hydroxy toluene  |                                                                                 | .0267  | .050    | .065    | .104    |
| Sample I containing .01% butylated hydroxy toluene   |                                                                                 | .0171  | .036    | .037    | .084    |
| Sample I containing .02% butylated hydroxy toluene   |                                                                                 | .0155  | .036    | .025    | .025    |
| Sample I containing .04% butylated hydroxy toluene   |                                                                                 | .0161  | .034    | .026    | .018    |

The stabilized epoxidized soybean oil samples also exhibited far greater compatibility in vinyl chloride formulations than the unstabilized control. While films prepared from polyvinyl chloride resin formulations plasticized with

oxirane determinations were made after 14, 21, and 28 days. The increasing effectiveness of the stabilizer in inhibiting loss of oxirane oxygen as increasing amounts are added can be seen.

TABLE IV

| Sample                                               | Percent Oxirane After Number of Days Indicated at 85° C. |         |         |         |
|------------------------------------------------------|----------------------------------------------------------|---------|---------|---------|
|                                                      | 0 days                                                   | 14 days | 21 days | 28 days |
| Sample I, epoxidized soybean oil (control)           | 7.02                                                     | 7.03    | 6.87    | 6.77    |
| Sample I containing .0025% butylated hydroxy toluene |                                                          | 7.03    | 6.93    | 6.89    |
| Sample I containing .005% butylated hydroxy toluene  |                                                          | 7.03    | 6.91    | 6.87    |
| Sample I containing .01% butylated hydroxy toluene   |                                                          | 7.05    | 6.98    | 6.91    |
| Sample I containing .02% butylated hydroxy toluene   |                                                          | 7.07    | 7.00    | 7.00    |
| Sample I containing .04% butylated hydroxy toluene   |                                                          | 7.07    | 7.00    | 7.00    |

cized with the control sample showed considerable exudation of the plasticizer films prepared from similar polyvinyl chloride resin formulations plasticized with the stabilized epoxidized oils were substantially free of exuded plasticizer.

60

## Example III

Epoxidized esters of 2-ethylhexyl alcohol (oxirane oxygen 4.9%) esterified with tall oil fatty acids were employed as the oxirane-containing composition and butylated hydroxy toluene was employed as the stabilizer in this test. Accelerated aging tests were carried out in the manner of the preceding examples and the stabilizing effect is noted in Tables V and VI, which follow.

TABLE V

| Sample                                                                                       | Percent Free Fatty Acid (as Acetic)<br>After Number of Days Indicated as 85° C. |        |         |         |         |
|----------------------------------------------------------------------------------------------|---------------------------------------------------------------------------------|--------|---------|---------|---------|
|                                                                                              | 0 days                                                                          | 7 days | 14 days | 21 days | 28 days |
| Epoxydized 2-ethylhexyl tallate (control)                                                    | .036                                                                            | .169   | .246    | .38     | .56     |
| Sample I containing .01% butylated hydroxy toluene                                           | .036                                                                            | .35    | .232    | .30     | .38     |
| Sample I containing .1% butylated hydroxy toluene                                            | .036                                                                            | .082   | .071    | .096    | .172    |
| Sample I refined with aqueous sodium hydroxide and containing .02% butylated hydroxy toluene | .036                                                                            | .016   | .034    | .026    |         |

Oxirane determinations for these samples were conducted and the results are as follows:

TABLE VI

| Sample                                                                                       | Percent Oxirane After Number of Days Indicated at 85° C. |         |         |         |
|----------------------------------------------------------------------------------------------|----------------------------------------------------------|---------|---------|---------|
|                                                                                              | 0 days                                                   | 14 days | 21 days | 28 days |
| Epoxidized 2-ethylhexyl tallate (control)                                                    | 4.90                                                     | 4.73    | -----   | 4.20    |
| Sample I containing .01% butylated hydroxy toluene                                           | 4.90                                                     | -----   | -----   | 4.52    |
| Sample I containing .1% butylated hydroxy toluene                                            | 4.90                                                     | -----   | 4.91    | 4.90    |
| Sample I refined with aqueous sodium hydroxide and containing .02% butylated hydroxy toluene | 5.00                                                     | -----   | 5.03    | -----   |

It can be seen that alkali refining of the epoxidized ester aids considerably in stabilizing effectiveness.

#### Example IV

The oxirane-containing material employed in this test is high-oxirane linseed oil having an oxirane oxygen value of 9.22%, an iodine value of 4, a Gardner color less than 1, and infrared absorptivity at 2.9 microns (corrected for background) of .020 maximum. The epoxidized linseed oil has a low polymer content and a low hydroxyl content, as illustrated by the infrared absorption. In addition, the low viscosity (8.8 poises) is further evidence of the low polymer content.

Varying amounts of butylated hydroxy toluene were added to this oil and the stabilizing effect as compared to a control sample having no stabilizer added was determined by free fatty acid content and oxirane oxygen values.

The two batches were worked on a 2-roll mill for 5 minutes at 330° F. with the roll speeds being adjusted to

50% and 60%. Small pieces, 6" x 6" were cut from the films obtained and these small pieces were placed in a preheated (345° F.) chrome mold. The mold was placed in a Carver Press so that the heating plates of the press were in contact with the mold. The contact pressure was maintained for 5 minutes, while the temperature was held at 345° F. and then the pressure was increased to 20,000 p.s.i. The mold was held under this pressure for 5 minutes. After cooling, the pieces were removed from the mold and placed in a Fadeometer for 100 hours. Examination of the films after 100 hours showed that the film prepared from the epoxidized oil containing no stabilizer exhibited some loss of gloss and some exudation, while the film prepared from the formulation having stabilized epoxidized oil was substantially free of exudation and was characterized by good gloss.

The stabilizers employed herein are compatible with other materials employed in vinyl halide resin formula-

TABLE VII

| Sample                                             | Percent Free Fatty Acid (as Acetic) After Number of Days Indicated at 85° C. |        |         |         |         |
|----------------------------------------------------|------------------------------------------------------------------------------|--------|---------|---------|---------|
|                                                    | 0 days                                                                       | 7 days | 14 days | 21 days | 28 days |
| Epoxidized linseed oil (control)                   | .018                                                                         | .051   | .083    | .107    | -----   |
| Sample I containing .02% butylated hydroxy toluene | .018                                                                         | .032   | .035    | .019    | -----   |

TABLE VIII

| Sample                                             | Percent Oxirane After Number of Days Indicated at 85° C. |        |         |         |         |
|----------------------------------------------------|----------------------------------------------------------|--------|---------|---------|---------|
|                                                    | 0 days                                                   | 7 days | 14 days | 21 days | 28 days |
| Epoxidized linseed oil (control)                   | 9.22                                                     | 9.16   | 9.10    | 8.92    | -----   |
| Sample I containing .02% butylated hydroxy toluene | 9.22                                                     | 9.18   | 9.23    | 9.20    | -----   |

Typical of the vinyl halide polymers with which the stabilized epoxidized fats are most useful are those polymers in which at least 50% of the monomer units prior to polymerization are vinyl halide units. This includes polyvinyl chloride, polyvinyl bromide, polyvinyl fluoride, polyvinylidene chloride, vinyl chloride-vinylidene, chloride copolymers, vinyl chloride, vinyl acetate copolymers as well as homopolymers and interpolymers of vinyl halides. Other monomers which may be copolymerized with vinyl halides include vinyl ketones such as vinyl butyl ketone, the acrylates and lower alkyl acrylates and alkacrylates as well as lower alkyl esters of maleic and fumaric acids.

#### Example V

A formulation containing the following ingredients:

|                                            | Parts |
|--------------------------------------------|-------|
| Polyvinyl chloride                         | 100   |
| Epoxidized soybean oil (oxirane oxygen 7%) | 40    |
| Zinc stearate                              | 0.25  |
| Mineral oil                                | 1     |

was prepared and a similar formulation was prepared containing the same ingredients in the same amounts, with the exception that stabilized epoxidized soybean oil was substituted for the unstabilized plasticizer. This stabilized oil contained .05% based on the weight of the oil of a stabilizer mixture made up of 20 parts propyl gallate, 10 parts citric acid, and 70 parts propylene glycol,

tions such as lubricants, heat stabilizers (such as the metal salts) and antistatic agents. The alkyl phenols can be employed alone or in combination to obtain the superior stabilization. In addition, stability enhancing materials can be employed with the phenolic stabilizers. These enhancing agents include citric acids, phosphoric acid, etc.

The stabilizers impart improved color stability to polyvinyl chloride resin compositions containing the stabilized oxirane-containing fatty materials. The improvement in color stability in the polyvinyl chloride compositions after formulation on extruders and after exposure to elevated temperatures is substantial. This improvement has been noted at low levels of the stabilizer around .01-1% and also at much higher levels in the range of up to 5%.

Obviously, many modifications and variations of the invention as hereinbefore set forth may be made without departing from the spirit and scope thereof and, accordingly, only such limitations should be imposed as are indicated in the appended claim.

We claim:

1. Esters of oxirane substituted higher fatty acids of 7-30 carbon atoms containing from about .0025% to about 5% of propyl gallate based on the weight of said esters.

2. The product of claim 1, wherein said ester is epoxidized soybean oil.

3,497,531

9

3. The product of claim 1, wherein said propyl gallate is in admixture with citric acid which together are present in an amount of about .0025% to about 5% based on the weight of said esters.

10

3,075,940 1/1963 Pazinski ----- 260—45.85 XR  
3,091,597 5/1963 Henriques ----- 260—23 XR  
3,125,592 3/1964 Nevin ----- 260—45.85

References Cited

5

841,890 7/1960 Great Britain.

UNITED STATES PATENTS

2,759,829 8/1959 Mattil et al. ----- 260—398.5  
2,772,170 11/1956 Hall ----- 260—398.5  
2,967,774 1/1961 Bell et al. ----- 99—163  
2,981,628 4/1961 Hall ----- 260—398.5  
3,060,121 10/1962 Orloff et al. ----- 252—48.2  
3,067,165 12/1962 Hudson ----- 127—37  
3,068,193 11/1962 Havens et al. ----- 260—348 XR  
3,071,560 1/1963 Fetscher et al. ----- 260—23 XR

15

260—23, 30.4, 45.8, 45.85, 45.95

FOREIGN PATENTS

OTHER REFERENCES

Junberg, W. G.: "Autoxidation and Antioxidants," vol. II, chapter 12, pp. 477—542, Interscience Publisher, 1962.

NORMA S. MILESTONE, Primary Examiner

U.S. Cl. X.R.